

## UNITED STATES PATENT OFFICE

2,414,491

## PHOTOGRAPHIC DEVELOPER

Vsevolod Tulagin, Phillipsburg, N. J., assignor to  
 General Aniline & Film Corporation, New York,  
 N. Y., a corporation of Delaware

No Drawing. Application January 27, 1945,  
 Serial No. 574,973

16 Claims. (Cl. 95—88)

1

The present invention relates to photographic developers which may be used for the production of black and white images but are of special interest for the production of dyestuff images and to a process of producing said dyestuff images by color-forming development.

Para-phenylene diamines and substituted para-phenylene-diamines have been used extensively as photographic developers, particularly for fine grain work. It is considered that the fine grain obtained with these developers is attributable to some solvent action on silver halide and a comparatively low reduction potential. Despite the desirable properties which are possessed by p-phenylenediamine and its N-alkyl substitution products, efforts are being continuously made to find other developers for black and white photographic work which show an improvement over the p-phenylenediamine and its N-alkyl substitution products, chiefly in regard to gradation and speed utilization of the photographic negative emulsions.

One of the methods which is widely used for the production of color images involves the so-called "color development" method. This method was devised by Fischer and is described in his United States Patent 1,102,028. The basis of this process involves the reaction of the oxidation products of a primary amino developer, preferably a dialkylamino-aniline in the presence of a color former whereby dyestuff images are produced in situ with the silver image. Upon removing the silver image by the use of a mild oxidizing agent such as a ferricyanide, followed by fixing with a thiosulfate bath, pure dyestuff images are obtained. The color formers which are employed in this method may be generally classified as phenols, primary aromatic amines and compounds containing a reactive methylene group such as acetoacetanilides, pyrazolones and the like. By a proper selection of the color formers, there may be produced upon color development the desired subtractive colors in a three-layer photographic film, i. e., yellow, magenta and cyan. The dyestuffs which are produced by this color-forming development method are of the type of azomethine and quinoneimine dyes.

I have now discovered that developers having properties superior to the conventionally employed p-phenylenediamine and its N-alkyl substitution products, are obtained by utilizing compounds which are aromatic amines, having a primary amino group and which contain on a ring carbon atom in o-position to the primary amino group a sulfonamido group, the primary amino

2

group being activated by a substituent, preferably a substituted amino group in p-position thereto. These compounds when used as developers in the production of black-and-white images give a fine grain and greater contrast than can be obtained with the conventional p-phenylenediamines. They also permit better speed utilization of the photographic negative emulsion.

In the color development method, the density of the dyestuff image is proportional to the amount of silver image produced on development. My new developers because of their more energetic action, yield denser silver images of greater contrast than can be obtained with the usually employed p-dialkylamino-anilines, and this, in turn, means that the density and contrast of the color images are likewise enhanced. With the new developers it is possible to obtain sufficiently saturated or dense dye images from a normal negative emulsion having low or medium contrast, high speed and the finest possible grain. It is therefore unnecessary to build up excessive contrast to obtain sufficient dye density at the sacrifice of emulsion speed, gradation, latitude and grain. This property is of the greatest importance in the production of negatives by direct color development of an exposed film or plate where a well graded dye image must be obtained at often prevailing low levels of exposure.

However, probably the most important property of the new developers when used in the color-forming development method is their ability to yield as the ultimate dyestuff of the color image an azine dye rather than the usually obtained azo-methine and quinoneimine dyes. While the azo-methine and quinoneimine dyestuff images heretofore obtained are generally satisfactory, they possess the disadvantages of being unstable to light and to acids and alkalies. Consequently, there is the danger that such dyestuff images will fade appreciably after long use or if exposed to atmosphere containing acid vapors.

It is accordingly an object of this invention to produce photographic developers in which the developing agent is an aromatic amine containing a primary amino group activated by a substituent in the p-position thereto and having a sulfonamido group in o-position to the primary amino group.

It is a further object of this invention to produce color developers capable of yielding azine dyes in color development comprising an aromatic amine having a primary amino group activated by a substituent in p-position thereto and having

## 3

a sulfonamido group in o-position to said primary amino group.

A further object of this invention is to produce azine dyestuff images by color-forming development.

A further object of this invention is a process of producing dyestuff images by color developing an exposed silver halide emulsion with an aromatic amine containing a primary amino group activated by a substituent in p-position thereto and having a sulfonamido group in o-position to the primary amino group in the presence of a color former.

It is a further object of this invention to provide a process of producing azine dyestuff images by color development of an exposed silver halide with an aromatic amine containing a primary amino group and a sulfonamido group in o-position to the primary amino group in the presence of a color former.

It is a further object of this invention to produce color developers containing a color former and as the developer an aromatic amine having a primary amino group activated by a substituent in p-position thereto and having in o-position to said amino group a sulfonamido group.

It is a further object of this invention to color develop a photographic silver halide emulsion containing a color former fast to diffusion by means of a developer comprising an aromatic amine having a primary amino group activated by a substituent in p-position thereto and having a sulfonamido group in o-position to the primary amino group.

Other and further important objects of the invention will become apparent as the description proceeds.

The developing agents which I contemplate may be generally characterized as aromatic amines containing a primary amino group and in o-position to said amino group a sulfonamido group derived from an aliphatic or aromatic sulfonyl compound, the primary amino group being activated by a nitrogen atom in p-position to said amino group. The compounds may be purely aromatic and of the type of p-phenylenediamines or they may have a fused-on heterocyclic nucleus, in which case the activating N-atom in p-position to the primary amino group forms part of the heterocyclic ring system. In other words, the compounds always have at least one ring, aromatic in nature, to which the primary amino, sulfonamido and activating N-atom are linked. Compounds of this general character may be formulistically represented as follows:



and



## 4

in which R is an aliphatic radical such as methyl, ethyl, propyl, butyl, amyl, vinyl, allyl, cyclopentyl, cyclohexyl, chlorbutyl, sulfoethane and the like, or an aromatic radical such as phenyl, naphthyl, sulfophenyl, alkoxyphenyl, i. e., methoxyphenyl, ethoxyphenyl and the like, chlorphenyl, toluyl, anisyl and the like, R1 represents hydrogen or an aliphatic or aromatic radical as illustrated above, R2 represents hydrogen, sulfo, or an aliphatic or aromatic radical as above, Y represents —N, —NH, —N-alkyl such as —N-methyl, —N-ethyl, —N-propyl and the like, and X represents the atoms necessary to complete a five- or six-membered heterocyclic ring system such as a thiazole, an imidazole, a dihydropyridine, an oxazole, or the like.

Examples of compounds which fall within the general classes referred to hereinabove are the following:



3-phenylsulfonamino-4-amino-diethylaniline



3-methylsulfonamino-4-amino-diethylaniline



3-methylsulfonamino-4-amino-6-methyl-diethylaniline



3-chlorbutylsulfonamino-4-amino-dimethylaniline



3-dodecylsulfonamino-4-amino-diethylaniline



4-amino-3-vinylsulfonamino-diethylaniline

5



3-ethylsulfonamino-4-amino-6-sulfodiethylaniline



3'-methoxy-3-phenylsulfonamino-4-amino-diethylaniline



6-butylsulfonamino-5-amino-benzoxazole



6-methylsulfonamino-5-amino-benzthiazole



7-methylsulfonamino-6-amino-1-N-methyl-dihydroquinazoline



1-ethyl-5-amino-6-benzenesulfonamino-iso-indazole



1-ethyl-6-ethylsulfonamino-5-amino-benzimidazole

The sulfonamido compounds of the present invention may be synthesized by various methods. For instance, the proper 3-alkyl or aryl-sulfonamino dialkyl-aniline may be nitrosated and the introso compound reduced to the required amine. Or such dialkylanilines may be nitrated and subsequently reduced. Furthermore, the prod-

6

ucts can be obtained by the reduction of an appropriate azo dye, for example:

5



The reduction of the azo dyes may be performed by subjecting the dye to the action of hydrogen in the presence of a hydrogenating catalyst such as platinum oxide, whereby the azo linkage is split and the amino group is formed.

It has been stated that the developers may be utilized to produce azine dyes. It has been ascertained that in general such dyes are formed when the color formers are phenols, naphthols, anthrois and the like, aromatic amines and perimidines. In some instances when employing alkylated amino phenols as the color formers, for example, 3-diethylaminophenol, quinoneimine dyes rather than azine dyes appear to be formed. It is also observed that with the acetoacetanilides, dyestuffs are produced on color forming development which cannot be definitely identified as azine dyes. It is true that the dyestuffs obtained with these compounds have a higher stability to mineral acids than most quinoneimine dyes. However, unlike the azines, they are slowly bleached by mineral acids and by dichromate bleaches and hence it cannot be said with assurance that they are azines.

The reaction by which the azine dyes are formed may be graphically represented by the following equation:

35



55

It will be noted that there is first formed the quinoneimine dye the same as when using the conventional p-dialkylamino-anilines. Subsequently, however, due to the presence of the sulfonamido group, ring closure ensues, with splitting off of the sulfonyl group yielding the desired azine compound. The reaction depending upon the particular components involved may take place spontaneously so that the formation of the quinoneimine is not observable as an independent reaction. In other cases, however, the ring closure to the azine dye may take hours or even days. The ring closure, however, can be facilitated or catalyzed by the utilization of acids such as hydrochloric, sulfuric, phosphoric and the like, or by the use of alkalies such as sodium hydroxide, potassium hydroxide, sodium carbonate and the like.

The developers herein described may be utilized to develop negative film, positive film, reversal film or paper prints. The developers may

be employed along with the color formers in the developer or the color formers may be located in the emulsion. In the latter event, it is advisable to render the color formers fast to diffusion and this may be accomplished either by the introduction of a substantive group or by the introduction of a molecular enlarging group such as a natural resin, a synthetic resin, a sterol, a carbohydrate, a terpene, or a long fatty chain. The last-named method is preferred and good results have been obtained when using as such long chain, radicals such as decyl, dodecyl, stearyl, oleyl and the like. The means by which the color formers may be rendered fast to diffusion are described in U. S. P. 2,178,612, 2,179,228, 2,179,238, 2,179,244, 2,179,239, 2,186,685, 2,186,719, 2,186,732, 2,186,733, 2,186,734, 2,186,849, 2,186,851, 2,186,852 and the like. The color formers may be located in emulsion layers of a multilayer film or a bi-pack, the color formers being selected so that subtractively colored dyestuff images are obtained in each of the layers.

When the color formers are located in the silver halide emulsion, the main ingredients of the color developer are the aromatic amine containing the sulfonamido group and an alkali. The color former of course is an essential ingredient when all of the reaction components are in the developer. The alkali which is employed may be sodium bicarbonate, sodium carbonate and the like. The developer may also contain other ingredients such as an alkali metal bromide, i. e., potassium bromide, a sulfite, i. e., sodium metabisulfite, etc.

In carrying out the process while using the new developing agents, the emulsion after the formation therein of a latent silver image is developed with said developing agent in the presence of a color former whereupon the film is rinsed and subjected to the action of a stop bath. This bath usually comprises a solution in water of an organic acid such as acetic acid or an acid salt such as sodium bisulfite. Following this treatment, the silver is removed by a ferricyanide bleach, thoroughly washed and fixed in an acid-hardening typo. After washing free from hypo, the film is dried, whereupon a photographic element containing pure dyestuff image results.

The following examples will serve to further explain the present invention, but it is to be understood that the invention is not restricted thereto. The parts are by weight, unless otherwise stated.

#### PREPARATION OF THE AROMATIC AMINES CONTAINING THE SULFONAMIDO GROUP

##### Example 1

Into a three-necked reactor equipped with a stirrer, a dropping funnel and a thermometer is introduced a solution of 55 parts of concentrated sulfuric acid in 2000 parts of water and to this solution are added 51 parts of 3-phenyl sulfonamino diethylaniline hydrochloride. The mixture is stirred until said hydrochloride goes into solution, whereupon it is cooled to  $-3^{\circ}$  C. using a freezing mixture of water and ice. 105 parts of sodium nitrite dissolved in 250 parts of water are added during a period of about 10 minutes. The mixture is then stirred for an hour at  $3^{\circ}$  C. and filtered. The wet solid thus obtained is stirred for about one-half hour with 245 parts of concentrated hydrochloric acid and then treated with a warm solution of 140 parts of

stannous chloride dissolved in 163 parts of concentrated hydrochloric acid. The mixture so produced is stirred for 15 minutes and then placed in an ice bath for a few hours. The crystalline material which precipitates is dried and dissolved in a hot mixture of 200 parts of water and 16.6 parts of a solution of 100 parts of stannous chloride in 233 parts of concentrated hydrochloric acid.

The mixture is decolorized by Nuchar, filtered and the filtrate is treated with a solution of 100 parts of stannous chloride in 233 parts of concentrated hydrochloric acid. This mixture is placed in an ice chamber for three hours, whereupon the white crystalline 3-phenyl sulfonamino-4-amino-diethylaniline stannochloride precipitates. It is washed with a little concentrated hydrochloric acid and dried. The yield is 63 parts. For convenience, this product will hereinafter be referred to as developing agent I.

##### Example 2

To a solution of 60 parts of 3-amino diethylaniline in 220 parts of anhydrous benzene are added dropwise and with agitation, 41 parts of methane sulfonyl chloride while maintaining the temperature below  $20^{\circ}$  C. The addition is complete after about  $\frac{3}{4}$  hour. The mixture is stirred for 1 hour and then treated with 12 parts of anhydrous pyridine and stirred over night at room temperature.

The thick slurry thus obtained is filtered and the precipitate is twice washed with 44 parts of anhydrous benzene. The resinous solid which results is boiled for 20 minutes with 118 parts of isopropyl alcohol and the mixture is then placed in the ice chest for several hours. The crystalline 3-methyl sulfonamino diethylaniline hydrochloride so obtained is isolated by filtration, washed with 118 parts of isopropyl alcohol and dried. There are obtained 84 parts of colorless crystals, representing a yield of 82 per cent.

28 parts of the 3-methyl sulfonamino diethylaniline hydrochloride are dissolved in 1000 parts of water and 47 parts of concentrated hydrochloric acid and the solution cooled to  $-5^{\circ}$  C. 7 parts of sodium nitrite in 15 parts of water are added dropwise to the cooled solution with agitation. After about 1 hour and a half, the suspension is filtered and the 4-nitroso-3-methyl sulfonamino diethylaniline hydrochloride so obtained is dried in a vacuum desiccator. There are obtained 29 parts of the product, representing a yield of 93.5 per cent.

A mixture of 135 parts of absolute alcohol, 30 parts of distilled water, 31 parts of 4-nitroso-3-methyl-sulfonamino diethylaniline hydrochloride and .2 to .3 part of platinum oxide is subjected to the action of hydrogen at 60 pounds gauge pressure. The reactor is then carefully opened and 13 parts of concentrated hydrochloric acid introduced. The air in the reactor is replaced by hydrogen and the contents thoroughly mixed. The suspension is filtered and the platinum is removed by washing with a solution of 12 parts of concentrated hydrochloric acid in 50 parts of water and the mixture filtered. The two filtrates are combined and evaporated to dryness at a pressure of 3 mm. at a temperature of  $98^{\circ}$  C. The residue is dissolved in 79 parts of absolute alcohol and the solution placed in an ice chest over night. There is thus obtained crystalline 3-methyl sulfonamino - 4 - amino-diethylaniline hydrochloride, which is washed to a light yellow color with absolute alcohol. 25.5 parts

of the product are obtained, representing a yield of 79.5 per cent. For convenience, this product hereinafter will be referred to as developing agent II.

*Example 3*

38.2 parts of methyl sulfonyl chloride are added dropwise to a solution of 50 parts of 2-methyl-5-amino-dimethylaniline and a small amount of pyridine in 264 parts of anhydrous benzene while agitating the solution. The addition takes about 20 minutes. After standing at room temperature for 1½ hours, the mixture is refluxed on a steam bath for 15 minutes and cooled with ice. The resulting crystalline solid is isolated by filtration, dried and heated to boiling with 158 parts of absolute alcohol. The mixture is cooled, whereupon 2-methyl-5-methylsulfonamino-dimethyl aniline hydrochloride precipitates. The precipitate is isolated by filtration and dried. 62.9 parts of the product are obtained, which represents a yield of 81.8 per cent. The product when analyzed showed:

Calculated

C: 45.52 45.34  
H: 6.46 6.47  
Cl: 13.2 13.38

A cold solution of 17 parts of sulfanilic acid (monohydrate), 4.7 parts of anhydrous sodium carbonate and 6.6 parts of sodium nitrite in 108 parts of water is added to a mixture of ice and 22 parts of concentrated hydrochloric acid. After about 1½ hours, the resulting diazonium solution is added slowly and with agitation to a mixture of 23.6 parts of 2-methyl-5-methyl sulfonamino-dimethylaniline and 7.9 parts of anhydrous sodium carbonate in 200 parts of water. The suspension is treated with 55 parts of 10% sodium hydroxide solution and allowed to stand for two days. The solution is then saturated with salt and made strongly acid with hydrochloric acid. The dye, which crystallized in long needles, was collected, washed with a little water and dried. 24.1 parts of the dye are obtained, which represents a yield of 65.7 per cent of the pure 2-methyl sulfonamino-4-dimethylamino-5-methyl azobenzene-4'-sulfonic acid.

14.5 parts of sodium hydrosulfite are added to a mixture of 12 parts of the above azo dye, 3.3 parts of anhydrous sodium acetate and 100 parts of water. The solution is then extracted five times with 16 parts of carbon tetrachloride and neutralized with sodium carbonate. The suspension thus obtained is extracted three times with 32 parts of carbon tetrachloride. The aqueous phase is discarded. The combined organic extracts are extracted successively with 78.75 parts, 26.25 parts and 15.75 parts of 5% hydrochloric acid solution in water. These acid solutions are evaporated to dryness at 98° C. under 3 mm. pressure and the residue is recrystallized from 32 parts of absolute alcohol. 2 parts of 2-methyl-4-amino-5-methyl sulfonamino-dimethylaniline dihydrochloride, representing a yield of 24.5 per cent is thus obtained. This product is hereinafter to be referred to as developing agent III.

*Example 4*

A solution of 20 parts of 1-ethyl-6-nitro isoindazole (prepared by the method of Witt-Noelting and Grandmaugen, Ber., 23, 3640) in 200 parts of ethyl alcohol is treated with 2-3 part of platinum oxide catalyst and reduced with hydrogen at 60 pounds gauge pressure until no more hydrogen is taken up.

The suspension is filtered and evaporated to dryness at reduced pressure. The residue is treated with 15 parts of anhydrous pyridine and again evaporated to dryness at reduced pressure. The residue is now dissolved in 100 parts of pyridine.

To the resulting solution, is added dropwise, with cooling and agitation, a mixture of 19.3 parts of benzenesulfonyl chloride and 45 parts of benzene. The temperature of the mixture is maintained at 15° C. during the addition. After stirring for 16 hours, the reaction mixture is evaporated to dryness at reduced pressure.

The residue is taken up in 50 parts of ethyl alcohol and added to 300 parts of 6 N hydrochloric acid. The resulting solution is warmed to 50-60° C., decolorized, cooled with ice, and neutralized with concentrated ammonium hydroxide.

The resulting suspension is held in an ice bath until the precipitate solidifies and is then filtered. The solid so obtained is dissolved in 50 parts of hot ethyl alcohol. The resulting solution is treated with hot water to incipient cloudiness, decolorized and cooled. The crystalline material so obtained is used without further purification. Yield—20 parts by weight.

To a solution of 15 parts of the above 1-ethyl-6-benzenesulfonamino isoindazole in 100 parts of glacial acetic acid and 20 parts of acetic anhydride is added dropwise and with agitation a solution of 3.2 parts of fuming nitric acid in 40 parts of glacial acetic acid. The temperature of the mixture is maintained at 60-70° C. during the addition and then for 25 minutes longer. The mixture is, finally, cooled and added to 200 parts of ice-water.

The crystalline solid so obtained is collected by filtration, washed with water and dissolved in a hot solution of 20 parts of sodium bicarbonate in 200 parts of water. The resulting red solution is decolorized and acidified with acetic acid. The precipitated yellow solid is collected by filtration and washed with water.

Said yellow solid is dissolved in 40 parts of boiling acetic acid and poured into 200 parts of boiling 6N sulfuric acid. The precipitated by-product of 1-ethyl-6-benzenesulfoamino-7-nitroisoindazole is collected by filtering the hot solution. The filtrate on cooling deposited long white needles of 1-ethyl-6-benzenesulfonamino-5-nitroisoindazole sulphate.

The isoindazole sulphate obtained above is dissolved in an excess of dilute sodium hydroxide and the free 1-ethyl-6-benzenesulfonamino-5-nitroisoindazole is precipitated by saturating the resulting solution with carbon dioxide. The substance is further purified by crystallization from acetic acid. Yield—7 parts (40% theory). The product when analyzed showed: Found, N: 15.98; calculated, N: 16.18. 1 part of the above nitroisoindazole is treated with 10 parts of 3N sodium hydroxide and 1 part of sodium hydrosulfite. The mixture is heated on a steam-bath until a pale yellow solution results. It is then cooled and saturated with carbon dioxide. The precipitated 1-ethyl-5-amino-6-benzenesulfonamino isoindazole is collected by filtration and thoroughly washed with water. This product will hereinafter be referred to as developing agent IV.

PREPARATION OF DEVELOPER SOLUTIONS

*Example 5*

|                    |       |
|--------------------|-------|
| Part I:            | Parts |
| Developing agent I | 7.5   |
| Water              | 300   |

## 11

After the developing agent has been completely dissolved, add

Parts  
Nuchar (a decolorizing carbon black) 2

The suspension is saturated with hydrogen sulfide gas. 5 parts of Nuchar are added, and the suspension filtered. The filtrate is boiled until it is free of hydrogen sulfide, whereupon 5 parts of sodium metabisulfite are added. If this solution is to be stored, it should be kept in a well-stoppered bottle.

Part II: Parts  
Water 800  
Sodium bicarbonate 30  
Potassium bromide .5

When the developer is to be used, one volume of part I is added to four volumes of part II, the solution boiled for a few minutes, and cooled to 18° C.

## Example 6

Part I is the same as part I of Example 5.

Part II: Parts  
Water 800  
Sodium carbonate (monohydrate) 60  
Potassium bromide .6

When this developer is to be used, one volume of part I is added to four volumes of part II.

## Example 7

Part I: Parts  
Water 250 35  
Developing agent II 3.5  
Sodium metabisulfite 3.5

Part II:  
The same as part II of Example 5.

When this developer is to be used, one volume of part I is added to four volumes of part II, the solution boiled for a few minutes and cooled to 18° C.

## Example 8

Part I is the same as part I of Example 7.  
Part II is the same as part II of Example 6.

When the developer is to be used, 1 volume of part I is added to 4 volumes of part II.

## Example 9

Part I: Parts  
Water 250 55  
Developing agent III 5  
Sodium metabisulfite 5

Part II:  
Same as part II of Example 6.

When this developer is to be used, 1 volume of part I is added to 4 volumes of part II.

## Example 10

Part I: Parts  
Developing agent IV 7.5  
Water 300

After the developing agent has been completely dissolved, add

Parts  
Nuchar 2

The suspension is saturated with hydrogen sulfide gas. Five parts of Nuchar are added and the suspension filtered. The filtrate is boiled until

## 12

it is free of hydrogen sulfide, whereupon five parts of sodium metabisulfite are added.

Part II: Parts  
Water 800  
Sodium bicarbonate 30  
Potassium bromide .5

When the developer is to be used, one volume of part I is added to four volumes of part II, the resulting solution boiled for a few minutes and cooled to 18° C.

## PROCESSING OF EMULSIONS WITH DEVELOPERS

## Example 11

5 parts of 1-hydroxy-2-naphthalimide are added to the developer of Example 5. A photographic silver bromide emulsion is exposed and subjected to the action of said developer for a period of 15 minutes. The film is rinsed and treated with a stop bath containing 1000 parts of water and 7.34 parts of glacial acetic acid. The emulsion is then treated with a bleach of the following composition:

Parts  
Water 1000  
Potassium ferricyanide 100  
Disodium phosphate 4  
Monopotassium phosphate 6

The film is thoroughly washed and is then fixed in an acid hardening hypo bath. After removal of the hypo by washing and drying of the film, a red magenta azine dyestuff image is obtained.

## Example 12

10 parts of N-methyl-1-hydroxy-2-naphthalimide are added to the developer of Example 6. An exposed silver bromide emulsion is developed in the developer for a period of 10-20 minutes and then processed as in Example 11. A red magenta azine dyestuff image is thus obtained.

## Example 13

45 10 parts of N-ortho-methoxy acetoacetanilide are added to the developer of Example 7. An exposed silver halide emulsion is developed in the developer and further processed as in Example 11. There is thus obtained a silver halide emulsion containing a yellow dyestuff image. The dyestuff of the image has a high stability to mineral acids but it is slowly bleached thereby. The exact constitution of the dyestuff has not been determined.

## Example 14

55 5 parts of 1,5-dihydroxynaphthalene are added to the developer of Example 8. An exposed silver halide emulsion developed in said developer and further processed as in Example 11 yields a red magenta azine dyestuff image.

## Example 15

60 10 parts of 2-methyl perimidine are added to the developer of Example 5. An exposed silver halide emulsion is developed in the resulting developer and processed as in Example 11. There is thus obtained a film having a blue azine dye-stuff image.

## Example 16

70 10 parts of 1,5-dihydroxynaphthalene are added to the developer of Example 9. An exposed silver halide emulsion is developed in this developer and then processed as in Example 11. A

red dyestuff image of an azine dye is thus obtained.

*Example 17*

4 parts of octadecyl-1-hydroxy-2-naphthoyl-amide are dissolved in 5 cc. of sodium hydroxide solution of 20 per cent strength and about 50 cc. of methanol and the resulting solution is added to 1000 parts of a photographic silver halide emulsion. The resulting emulsion is coated on film, exposed and developed with the developer of Example 5. The film is then further processed as in Example 11. There is thus obtained a red magenta azine dyestuff image.

*Example 18*

1 kilo of a silver bromide emulsion is mixed with an aqueous solution of 15 parts of the sodium salt of 4"-stearyl-amino benzoyl-3"-aminobenzenesulfonyl-1-amino-8-hydroxynaphthalene-3,6-disulfonic acid. The emulsion is coated on a support to form a photographic silver halide emulsion layer.

The emulsion is exposed and developed with the developer of Example 5. After development, the film is processed as in Example 11. There is thus obtained a red magenta azine dyestuff image.

*Example 19*

1 kilo of a silver bromide emulsion is mixed with an aqueous solution of 15 parts of the sodium salt of 1-hydroxynaphthalene-2'-methyl-3'-stearyl-amino-anilide-5'-sulfonic acid. The emulsion is coated on a support to form a photographic silver halide emulsion layer.

The emulsion is exposed and developed with the developer of Example 6 and then further processed as in Example 11. A red azine dyestuff image is thus obtained.

The following table indicates the results obtained while utilizing the aforementioned developers with other color-formers:

bleaches. These azine dyes because of their stability have marked advantages over the usual azomethine and quinoneimine dyes.

Modifications of the invention will occur to persons skilled in the art and I therefore do not intend to be limited in the patent granted except as necessitated by the prior art and the appended claims.

I claim:

1. A photographic developer comprising an aqueous alkaline solution of a compound selected from the class consisting of those of the formulae:



35 in which R is selected from the class consisting of aliphatic and aromatic radicals, R<sub>1</sub> is selected from the class consisting of hydrogen, aliphatic and aromatic radicals, R<sub>2</sub> is selected from the class consisting of hydrogen, sulfo, aliphatic and aromatic radicals, Y is selected from the class consisting of -N-, -NH-, -N-alkyl, and X repre-

| Color former                                        | Developer | Color         | Type dye |
|-----------------------------------------------------|-----------|---------------|----------|
| 1-hydroxy-2-naphthalimide                           | Ex. 7     | Red magenta   | A        |
| N-methyl-1-hydroxy-2-naphthalimide                  | Ex. 8     | do            | A        |
| N-methyl-1-hydroxy-2-naphthalimide-4'-sulfonic acid | Ex. 5     | do            | A        |
| Do                                                  | Ex. 8     | do            | A        |
| 1,5-dihydroxynaphthalene                            | Ex. 6     | do            | A        |
| 1-hydroxy-2-naphthalimide                           | Ex. 9     | Orange        | A        |
| β-[amino-2-(7-hydroxynaphthyl)] crotonic acid       | Ex. 5     | Magenta       | A        |
| Do                                                  | Ex. 7     | do            | A        |
| Pyrocatechol                                        | Ex. 6     | do            | A        |
| Do                                                  | Ex. 7     | do            | A        |
| 8-methanesulfonamino-1-naphthol                     | Ex. 5     | do            | A        |
| 8-benzenesulfonamino-1-naphthol                     | Ex. 5     | Violet        | A        |
| Benzensulfonyl H acid                               | Ex. 5     | Reddish blue  | A        |
| 4-hydroxybenzearbazole (1,2)-2-sulfonic acid        | Ex. 6     | do            | A        |
| 1,8-naphthylenediamine                              | Ex. 6     | do            | A        |
| 2,5-dihydroxydiphenyl                               | Ex. 5     | Magenta       | A        |
| 3-allyl rhodanine                                   | Ex. 6     | do            | S        |
| 3-diethylaminophenol                                | Ex. 5     | Blue          | S        |
| Acetoacetanilide                                    | Ex. 6     | Yellow        | Q        |
| Do                                                  | Ex. 8     | do            | S        |
| o-Methoxyacetacetanilide                            | Ex. 6     | do            | S        |
| 8-acetamino-1-naphthol                              | Ex. 5     | Blue          | S        |
| Phenyl J-acid                                       | Ex. 6     | Violet        | A        |
| 1-anthryl-glycine                                   | Ex. 5     | Magenta       | A        |
| Diphenyl E-acid                                     | Ex. 5     | Green         | S        |
| 2-(2'-carboxyphenyl)-perimidine                     | Ex. 5     | Greenish blue | A        |
| 2-(3'-nitro-2'-carboxyphenyl)-perimidine            | Ex. 5     | Magenta       | A        |
| 2-perimidylacrylic acid                             | Ex. 5     | Blue          | A        |
| Phenol                                              | Ex. 9     | Yellow        | S        |
| o-Cresol                                            | Ex. 9     | Red           | A        |

A=azine dye.

Q=quinoneimine or azomethine.

S=uncertain—dyes in this class show a high stability to mineral acids but are slowly bleached by them. The same is true with "dichromate bleach."

The azine dyestuff images which are produced as above are, as stated, stable to mineral acids and strong alkalies. Furthermore, they are not affected by sulfuric acid nor by dilute acid dichromates such as are employed as dichromate bleach.

sents the atoms necessary to complete a ring system selected from the class consisting of 5- and 6-membered heterocyclic ring systems.

2. A color developer comprising an alkaline solution of a color former and a compound se-

15

lected from the class consisting of those of the formulae:



in which R is selected from the class consisting of aliphatic and aromatic radicals, R<sub>1</sub> is selected from the class consisting of hydrogen, aliphatic and aromatic radicals, R<sub>3</sub> is selected from the class consisting of hydrogen, sulfo, aliphatic and aromatic radicals, Y is selected from the class consisting of -N, -NH, -N-alkyl, and X represents the atoms necessary to complete a ring system selected from the class consisting of 5- and 6-membered heterocyclic ring systems.

3. A color developer as defined in claim 2 in which there is present an alkali metal sulfite.

4. A photographic developer comprising an alkaline solution of 3-phenyl sulfamino-4-amino-diethylaniline.

5. A photographic developer comprising an alkaline solution of 3-methyl sulfonamino-4-amino-diethylaniline.

6. A photographic developer comprising an alkaline solution of 2-methyl-4-amino-5-methylsulfonamino-dimethylaniline.

7. A color developer comprising an alkaline solution of 1-hydroxy-2-naphthylanide and 3-phenylsulfonamino-4-amino-diethyl-aniline.

8. A color developer comprising an alkaline solution of 1,5-dihydroxynaphthalene and 3-methyl-sulfonamino-4-amino-diethylaniline.

9. A color developer comprising an aqueous alkaline solution of 2-methyl perimidine and 3-phenyl-sulfonamino-4-amino-diethylaniline.

10. The process of producing photographic color images which comprises subjecting an exposed silver halide emulsion in the presence of a color former to the action of a developer containing as the developing agent a compound selected from the class consisting of those of the following formulae:



and

16

in which R is selected from the class consisting of aliphatic and aromatic radicals, R<sub>1</sub> is selected from the class consisting of hydrogen, aliphatic and aromatic radicals, R<sub>3</sub> is selected from the class consisting of hydrogen, sulfo, aliphatic and aromatic radicals, Y is selected from the class consisting of -N, -NH, -N-alkyl, and X represents the atoms necessary to complete a ring system selected from the class consisting of 5- and 6-membered heterocyclic ring systems.

11. The process of producing azine photographic dyestuff images which comprises subjecting an exposed silver halide emulsion in the presence of a color former selected from the class consisting of phenols, aromatic amines and perimidines, to the action of a developer containing as the developing agent a compound selected from the class consisting of those of the following formulae:



20 and



in which R is selected from the class consisting of aliphatic and aromatic radicals, R<sub>1</sub> is selected from the class consisting of hydrogen, aliphatic and aromatic radicals, R<sub>3</sub> is selected from the class consisting of hydrogen, sulfo, aliphatic and aromatic radicals, Y is selected from the class consisting of -N, -NH, -N-alkyl, and X represents the atoms necessary to complete a ring system selected from the class consisting of 5- and 6-membered heterocyclic ring systems.

12. The process of producing an azine dyestuff image which comprises subjecting an exposed silver halide emulsion to the action of a color developer containing 1-hydroxy-2-naphthylanide as the color former and 3-phenyl sulfonamino-4-amino-diethylaniline as the developing agent.

13. The process of producing azine dyestuff images which comprises subjecting an exposed silver halide emulsion to the action of a developer containing 2-methyl perimidine as the color former and 3-phenyl sulfonamino-4-amino-diethylaniline as the developing agent.

14. The process of producing azine dyestuff images in a photographic silver halide emulsion which comprises exposing the emulsion and developing the same in a color developer containing 1,5-dihydroxynaphthalene as the color former and 3-methyl sulfonamino-4-amino-diethylaniline as the developing agent.

15. The composition as defined in claim 1 wherein there is present an alkali metal sulfite.

16. The process as defined in claim 11 wherein there is present an alkali metal sulfite.